

## UNITED STATES PATENT OFFICE

2,082,936

DETERGENTS AND METHOD OF MAKING  
THE SAMEChester L. Baker, Berkeley, Calif., assignor to  
Philadelphia Quartz Company, Philadelphia,  
Pa., a corporation of PennsylvaniaNo Drawing. Application June 21, 1934,  
Serial No. 731,642

7 Claims. (Cl. 87—5)

This invention relates to detergent compositions as well as to a method of producing them. More specifically it relates to detergent compositions which include a mixture of crystalline alkali metal silicate such, for example, as sodium metasilicate and a boron containing compound as well as to a method for producing them.

Before proceeding with a detailed description of the nature and objects of the invention I should like to point out that ordinary borax ( $\text{Na}_2\text{B}_4\text{O}_7 \cdot 10\text{H}_2\text{O}$ ), while long used in industry as a fungicide and bactericide, is somewhat too weak an alkali to be used as a general detergent. In the citrus industry, therefore, it has heretofore been customary, by way of example, first to wash the fruit in an alkaline detergent solution in order to remove adhering dirt, after which it is often further treated by dipping it into a solution of ordinary borax ( $\text{Na}_2\text{B}_4\text{O}_7 \cdot 10\text{H}_2\text{O}$ ) in order to inhibit the growth of blue mold and other fungi upon the skin of the fruit during storage. This procedure, of course, involves two separate steps, first the cleaning step and then the disinfecting step. Similar situations arise in other industries.

I should also like to point out that the alkali metal silicates including particularly sodium metasilicate, while good detergents, are somewhat too caustic for uses which bring them into contact with citrus or pomaceous fruits or with human hands. Furthermore, if used at temperatures or concentrations which are too high they may also attack certain of the softer metals.

I have discovered that the fungicidal properties of borax can be combined with the detergent properties of the alkali metal silicates, particularly sodium metasilicate, to form a composition of matter which can be used for carrying out both washing and sterilizing operations simultaneously and the primary object of my invention is to provide a composition of matter of this nature which I shall term a fungicidal detergent.

With the foregoing in mind the objects of my invention may be stated in greater detail as follows: (1) the provision of a fungicidal detergent which possesses not only the high detergent value of sodium metasilicate but also the fungicidal and bactericidal properties of borax; (2) the provision of a detergent of the character specified which is extremely mild in its action on the skin and much less corrosive in its effect on the so-called softer metals such, for example, as aluminum and tin; (3) the provision of a novel method for the production of my improved composition of matter by means of which the mixture of the ingredients is so thoroughly and intimately ef-

fected as to preclude all possibility of segregation or separation of the constituents; (4) the provision of a product of the character described which will remain stable in storage and which can be ground to a dry granular or powdery condition.

The foregoing objects, together with such other objects as may appear hereinafter or are incident to my invention, can be attained in the following manner, although I wish it to be distinctly understood that the examples given while representing preferred procedure, are not to be taken as limitations upon the generic nature of the invention inasmuch as it will be perfectly clear to those skilled in the art that many variations might be adopted without departing from the spirit of the invention.

When ordinary borax ( $\text{Na}_2\text{B}_4\text{O}_7 \cdot 10\text{H}_2\text{O}$ ) is mixed with any one of the hydrates of sodium metasilicate, the mixture, after a comparatively short time, becomes either fluid or gummy in character and, therefore, unsuitable as an article of commerce. I have discovered, however, that if the lower hydrate of sodium tetraborate,  $\text{Na}_2\text{B}_4\text{O}_7 \cdot 5\text{H}_2\text{O}$ , is mixed with a compatible hydrate of sodium metasilicate such mixture will remain substantially dry and stable in storage and also that if ordinary borax is first converted into sodium metaborate, such metaborate may be mixed with sodium metasilicate to produce a dry stable product providing compatible hydrates of these two salts are chosen for use in the mixture.

It will be obvious that the requirements for stability in the several different mixtures are dependent upon the individual peculiarities of the crystalline compounds comprising a given mixture, the melting points and transition points of the various possible hydrates, possible chemical reactions with each other, and conditions requisite for phase equilibria. I have found, however, that the following combinations yield substantially dry, stable mixtures:

$\text{Na}_2\text{SiO}_3 \cdot 6\text{H}_2\text{O}$  and  $\text{Na}_2\text{B}_4\text{O}_7 \cdot 5\text{H}_2\text{O}$   
 $\text{Na}_2\text{SiO}_3 \cdot 5\text{H}_2\text{O}$  and  $\text{Na}_2\text{B}_4\text{O}_7 \cdot 5\text{H}_2\text{O}$   
 $\text{Na}_2\text{SiO}_3 \cdot 9\text{H}_2\text{O}$  and  $\text{NaBO}_2 \cdot 4\text{H}_2\text{O}$   
 $\text{Na}_2\text{SiO}_3 \cdot 5\text{H}_2\text{O}$  and  $\text{NaBO}_2 \cdot 2\text{H}_2\text{O}$   
 $\text{Na}_2\text{SiO}_3 \cdot 5\text{H}_2\text{O}$  and  $\text{NaBO}_2 \cdot \text{H}_2\text{O}$

For many uses a mechanical mixture of the two salts may be made. By way of example, 50 or more parts of sodium metasilicate hexahydrate,  $\text{Na}_2\text{SiO}_3 \cdot 6\text{H}_2\text{O}$  may be mixed by any suitable method with 50 or more parts of sodium tetraborate pentahydrate,  $\text{Na}_2\text{B}_4\text{O}_7 \cdot 5\text{H}_2\text{O}$ , and such mixtures will remain stable so long as they

are protected from the air. While such mechanical mixtures constitute an important part of my invention, I prefer wherever possible to crystallize the two salts together in the form of a hard brittle cake which can then be ground to a granular stable condition. This procedure prevents the possibility of segregation or separation of the individual constituents. Such a product is characterized by substantially complete crystallization of the constituents so that no uncrystallized water or mother liquor remains.

It is, therefore, another object of this invention to produce a hard brittle cake containing a mixture of sodium metasilicate and sodium borate which may be ground to what is an apparently dry, stable, granular or powdery condition.

A simultaneously crystallized mixture of this nature may be obtained by proceeding in general 20 as follows:

A mixture is prepared which is calculated to satisfy the chemical requirements of the desired composite product and crystallization of this mixture is effected in a manner which will convert 25 the entire mass into a hard brittle cake which can be ground to produce a stable granular product.

However, in some instances this end cannot be directly attained since the temperature of the mixture as well as the composition of the liquid 30 phase at any moment will determine the particular salt or salt hydrate which is likely to crystallize out so that unless especial precautions are employed, which will be described hereinbelow, the resulting product may not always be the desired one. In general, it may be stated that the mixture should be caused to crystallize within the temperature range of conditions where the desired crystalline compounds are in equilibrium and where they will crystallize from the prepared mixture without the formation of undesired crystalline compounds. If sufficient attention is not given to these details the resulting product will not be of the character desired. For instance, if one of the salts were to crystallize 45 with a lower degree of hydration the product would contain uncrystallized water and would be soft and fudge-like in consistency instead of hard and brittle as desired.

To more fully illustrate the difficulty just 50 discussed, I should like to point out that if one mixes directly a solution of silicate of soda with sufficient caustic soda and borax and evaporates sufficient water so that the resultant solution satisfies the chemical requirements of a mixture 55 of 50 parts of sodium metaborate tetrahydrate ( $NaBO_2 \cdot 4H_2O$ ) and 50 parts of sodium metasilicate nonahydrate ( $Na_2SiO_3 \cdot 9H_2O$ ) and then attempts to crystallize the mass by seeding, cooling and vigorous agitation, he will likely crystallize 60 lower hydrates than those desired, so that the product will be soft in consistency like fudge candy instead of hard and brittle. Such a product, of course, cannot be ground to a dry, free-flowing condition, and is, therefore, not suitable 65 for commercial purposes. Furthermore, it is not stable.

The reason for the undesired results mentioned in the preceding paragraph is to be found in the fact that there exists a transition point between 70  $NaBO_2 \cdot 4H_2O$  and  $NaBO_2 \cdot 2H_2O$  at a temperature of about  $55^\circ C$ . This means that a solution which would crystallize out  $NaBO_2 \cdot 2H_2O$  at a temperature above  $55^\circ C$ . must be crystallized at a temperature below  $55^\circ C$ . If  $NaBO_2 \cdot 4H_2O$  is to be obtained. Likewise, there is a transition point

between  $Na_2SiO_3 \cdot 6H_2O$  and  $Na_2SiO_3 \cdot 9H_2O$  at  $46.4^\circ C$ . so that if the latter compound is desired a solution of sodium metasilicate should be crystallized below  $46.4^\circ C$ . If one wishes, therefore, to crystallize a mixture of  $NaBO_2 \cdot 4H_2O$  and  $Na_2SiO_3 \cdot 9H_2O$ , he must bring about crystallization below  $55^\circ C$ . and also below  $46.4^\circ C$ . and if the temperature of the crystallizing mass tends to go above  $46.4^\circ C$ ., artificial cooling must be resorted to.

By way of specific example the following procedure may be followed in connection with the production of an intimate mixture of sodium metasilicate nonahydrate and sodium metaborate tetrahydrate. I wish it to be distinctly understood, however, that I do not wish to be limited to the exact proportions or procedure outlined as it is quite obvious that certain variations may be adopted without departing from the spirit or scope of the invention.

*Example for the preparation of an intimate mixture of  $Na_2SiO_3 \cdot 9H_2O$  and  $NaBO_2 \cdot 4H_2O$*

To 428 parts by weight of a solution of silicate of soda containing 18.5%  $Na_2O$  and 37%  $SiO_2$  25 is added 148.2 parts of caustic soda containing 76%  $Na_2O$  and then 250.3 parts of water is added. The solution thus formed should preferably be cooled sufficiently so that upon the addition of 173.5 parts of borax ( $Na_2B_4O_7 \cdot 10H_2O$ ) the temperature of the mass is below  $46.4^\circ C$ . The mass is then seeded with 25 parts of crystalline  $NaBO_2 \cdot 4H_2O$  and 75 parts of crystalline

$Na_2SiO_3 \cdot 9H_2O$ .

The mixture is then agitated and cooled until it becomes quite thick in consistency. During this process, care must be taken to keep the temperature of the mass below  $46.4^\circ C$ . The thickened mass is then allowed to cool in any suitable container. The hard cake thus formed may be ground to yield a dry, granular, free-flowing, stable product.

In carrying out the above example it is not imperative that the temperature of the mixture 45 be below  $46.4^\circ C$ . immediately after the addition of the borax, but in case it is higher the solution should be cooled to  $46.4^\circ C$ . with a minimum of agitation so as not to crystallize undesired hydrates.

I have further discovered that the desired mixture may be prepared if a solution of the desired sodium metasilicate is first prepared and crystallization thereof initiated and promoted to some extent before the required borax and caustic 55 soda are added. An example of this method is given below.

*Example for the preparation of an intimate mixture of  $Na_2SiO_3 \cdot 9H_2O$  and  $NaBO_2 \cdot 4H_2O$  where crystallization of the sodium metasilicate is begun before the borax and caustic soda are added*

583 pounds of a solution of silicate of soda containing 29 percent  $SiO_2$  and 8.9 percent  $Na_2O$  65 is run into a vessel which is equipped with a heavy agitator and a jacket for heating or cooling. 162 pounds of caustic soda is then added, brought into solution, and the solution thus formed is cooled to  $45^\circ C$ . 50 pounds of  $Na_2SiO_3 \cdot 9H_2O$  is 70 then added and the mass cooled and agitated until it becomes fairly thick and opaque. This indicates the formation of crystals of  $Na_2SiO_3 \cdot 9H_2O$ . At this stage is added a mixture comprising 592 pounds of borax and 125 pounds of caustic soda. 75

In some cases it may be necessary to add this mixture a little at a time, as it is important that the temperature does not go above 46.4° C. at this stage. When the addition is complete, 86 5 pounds of water are added and when the mass has again become homogeneous, 50 pounds of NaBO<sub>2</sub>.4H<sub>2</sub>O. Agitation and cooling is continued until the mass has become quite thick. It is then discharged from the mixer into any suitable 10 container. As the mass cools it will become hard and may be ground to produce a dry, stable, granular product.

*Method of preparing a mixture of Na<sub>2</sub>SiO<sub>3</sub>.9H<sub>2</sub>O and NaBO<sub>2</sub>.4H<sub>2</sub>O*

15 To 2250 grams of a solution of silicate of soda containing 28.82% SiO<sub>2</sub> and 8.84% Na<sub>2</sub>O are added 620 grams of caustic soda containing 76% Na<sub>2</sub>O and 630 grams of water. The solution 20 formed is then cooled to any convenient temperature below 55° C. At a temperature above 55° C. NaBO<sub>2</sub>.4H<sub>2</sub>O transforms into NaBO<sub>2</sub>.2H<sub>2</sub>O and since the former compound is desired, it is necessary to maintain the temperature below 25 55° C. To the solution is then added 1850 grams of borax (Na<sub>2</sub>B<sub>4</sub>O<sub>7</sub>.10H<sub>2</sub>O) and 390 grams caustic soda containing 76% Na<sub>2</sub>O. This addition is brought into solution by stirring, care being taken to prevent the temperature rising above 55° C. 30 The mass is then placed upon the two primary rolls of an ink grinding roll mill and 100 grams of Na<sub>2</sub>SiO<sub>3</sub>.9H<sub>2</sub>O and 100 grams of NaBO<sub>2</sub>.4H<sub>2</sub>O added for seed. The mixture is ground for about one minute and then discharged from the 35 machine as a white, opaque material which solidifies almost immediately to a hard brittle product which when ground will remain dry, free-flowing and stable upon storage. The product will consist of a definite mixture of NaBO<sub>2</sub>.4H<sub>2</sub>O and 40 Na<sub>2</sub>SiO<sub>3</sub>.9H<sub>2</sub>O.

In the above example it is advisable to continuously cool the rolls of the mill by artificial means so that the temperature of the mass will be brought to and maintained at a temperature 45 below 46.4° C. and thus insure the crystallization of the desired hydrates as well as facilitating crystallization by removing the heat liberated.

In the preparation of an intimately crystallized mixture of sodium metasilicate pentahydrate (Na<sub>2</sub>SiO<sub>3</sub>.5H<sub>2</sub>O) and sodium metaborate dihydrate (NaBO<sub>2</sub>.2H<sub>2</sub>O) it is of course necessary that crystallization be effected below the melting point of Na<sub>2</sub>SiO<sub>3</sub>.5H<sub>2</sub>O (72° C.) as well as 50 below the transition point between NaBO<sub>2</sub>.2H<sub>2</sub>O and NaBO<sub>2</sub>.4H<sub>2</sub>O. This transition point is not accurately known, but in practice good results may be had by preparing the mixture to be crystallized at a temperature below 65° C. By way 55 of example I might prepare an intimately crystallized mixture as follows:

*Example for the preparation of an intimately crystallized mixture of Na<sub>2</sub>SiO<sub>3</sub>.5H<sub>2</sub>O and NaBO<sub>2</sub>.2H<sub>2</sub>O*

65 To 1241 parts by weight of a solution of silicate of soda containing 29% SiO<sub>2</sub> and 8.9% Na<sub>2</sub>O is added 344 parts of caustic soda containing 76% Na<sub>2</sub>O and the solution thus formed evaporated 70 to a weight of 1272 parts. The hot solution should test just under 63° Baumé and should have a chemical composition corresponding to that of the formula Na<sub>2</sub>SiO<sub>3</sub>.5H<sub>2</sub>O. This solution is then cooled to a temperature of 72° or under, seeded 75 with 50 pounds of Na<sub>2</sub>SiO<sub>3</sub>.5H<sub>2</sub>O and agitated

and cooled until crystallization has well started and the mass has become white and opaque. 400 parts of finely ground NaBO<sub>2</sub>.2H<sub>2</sub>O is then mixed in and mixing and cooling continued as long as practicable. It may then be discharged into any 5 suitable container. Upon cooling, the mass will be found to be hard and brittle and may be ground to a dry, free-flowing and stable condition.

While the above example represents my preferred method for making an intimately crystallized mixture of Na<sub>2</sub>SiO<sub>3</sub>.5H<sub>2</sub>O and NaBO<sub>2</sub>.2H<sub>2</sub>O, it is possible to crystallize the two compounds more or less simultaneously as set forth in the following example.

*Example for the preparation of an intimately crystallized mixture of Na<sub>2</sub>SiO<sub>3</sub>.5H<sub>2</sub>O and NaBO<sub>2</sub>.2H<sub>2</sub>O*

To 1241 parts by weight of a solution of silicate of soda containing 29% SiO<sub>2</sub> and 8.9% Na<sub>2</sub>O is 20 added 344 parts of caustic soda containing 76% Na<sub>2</sub>O and the solution thus formed evaporated to a weight of 1272 parts. The hot solution should test just under 63° Baumé and should have a chemical composition corresponding to that of the 25 formula Na<sub>2</sub>SiO<sub>3</sub>.5H<sub>2</sub>O. This solution is then cooled to a temperature of 70° C. or under, seeded with 50 pounds of Na<sub>2</sub>SiO<sub>3</sub>.5H<sub>2</sub>O and agitated while maintaining the temperature above 55° C. When the mass has become quite thick and 30 opaque, one should add 36 parts of water, 81.5 parts of caustic soda containing 76% Na<sub>2</sub>O and 291 parts of Na<sub>2</sub>B<sub>4</sub>O<sub>7</sub>.5H<sub>2</sub>O. When this has been well mixed in, the temperature is adjusted if necessary to a value between 55° C. and 72° C. 35 50 parts of NaBO<sub>2</sub>.2H<sub>2</sub>O are then added for seed, and mixing with cooling continued as long as practicable. The doughy mass is then discharged from the mixer and allowed to cool. When cool it will be found to be hard and brittle and may 40 be ground to a stable granular or powdery condition.

By following the general method of the foregoing examples, it is quite possible to prepare mixtures with widely different proportions of 45 sodium metasilicate to sodium metaborate. Furthermore, the raw materials employed in the production of the desired products may have different characteristics, i. e., the silicates of soda may vary and also the borates. In addition the desired 50 end product may be obtained through the use of boric acid and caustic soda with the requisite amount of water instead of with the borax specified. Many other variations of a similar nature will occur to those skilled in the art.

In connection with all of the examples set forth above I wish to direct attention to the fact that it may not always be necessary to resort to seeding in order to initiate crystallization because in some instances I have found that crystallization 55 begins spontaneously when the proper conditions are established.

I claim:—

1. An alkaline detergent comprising an intimately crystallized mixture of sodium metasilicate nonahydrate and sodium metaborate tetrahydrate.

2. An alkaline detergent comprising an intimately crystallized mixture of sodium metasilicate pentahydrate and sodium metaborate dihydrate.

3. A method of preparing a mixture of sodium metasilicate nonahydrate and sodium metaborate tetrahydrate which includes the following steps:

(a) Preparation of a solution calculated to 75

satisfy the chemical requirements of sodium metasilicate nonahydrate.

(b) Adding sufficient borax, caustic soda and water to satisfy the chemical requirements of the desired metaborate.

(c) Cooling the mass to a temperature below 46.4° C.

(d) Seeding with crystals of sodium metasilicate nonahydrate and sodium metaborate tetrahydrate.

(e) Agitating the mass while maintaining the temperature of the crystallizing mass at a point below the melting temperature of both of the desired salts.

15 4. A method of preparing an intimately crystallized mixture of sodium metasilicate pentahydrate and sodium metaborate dihydrate which includes the following steps:

(a) Preparation of a solution having the chemical composition corresponding to the formula  $Na_2SiO_3 \cdot 5H_2O$ .

(b) Cooling the solution to a temperature of 70° C. or slightly thereunder and seeding with crystalline  $Na_2SiO_3 \cdot 5H_2O$ .

25 (c) Adding sodium tetraborate and caustic soda in the proportions required to form the desired sodium metaborate dihydrate.

(d) Holding the temperature of the mass between a temperature of 55° C. and 72° C. and 30 effecting crystallization thereof.

5. A method of preparing a mixture of sodium metasilicate nonahydrate and sodium metaborate tetrahydrate which includes the following steps:

35 (a) Preparation of a solution calculated to satisfy the chemical requirements of sodium metasilicate nonahydrate.

(b) Cooling the solution and initiating crystallization of sodium metasilicate nonhydrate.

40 (c) Adding the ingredients required to produce the composition of the desired mixture with further cooling, if necessary, to bring the temperature below 46.4° C., and

45 (d) Initiating crystallization of sodium metaborate tetrahydrate while maintaining the temperature below 46.4° C.

6. The method of preparing a dry stable mixture of sodium metasilicate pentahydrate and sodium metaborate dihydrate which comprises the following steps:

(a) Preparation of a solution calculated to satisfy the chemical requirements of sodium metasilicate pentahydrate;

(b) Cooling the solution to and maintaining it at a temperature between about 55° C. and 70° C.;

(c) Initiating crystallization of sodium metasilicate pentahydrate and permitting it to continue until the mass becomes fairly thick;

(d) Adding the ingredients required to produce the composition of the desired mixture accompanied with further cooling, if necessary, to maintain the said temperature;

(e) Initiating crystallization of sodium metaborate dihydrate; and

(f) Agitating and permitting the entire mass to cool and form a hard, grindable cake.

20 7. The method of preparing a dry, stable mixture of a desired hydrated sodium metasilicate and a compatible hydrated sodium metaborate as herein disclosed which comprises the following steps:

(a) Preparation of a solution calculated to satisfy the chemical requirements of the desired sodium metasilicate hydrate;

(b) Initiating crystallization of the said sodium metasilicate hydrate and permitting it to continue until the mass becomes fairly thick;

(c) Adding the ingredients required to produce the composition of the desired compatible sodium metaborate hydrate while cooling, if necessary, to maintain the temperature below the melting point 35 of the desired sodium metasilicate hydrate; and

(d) Initiating crystallization of the compatible sodium metaborate hydrate with further cooling, if necessary, to maintain the temperature below the melting temperature of the said crystalline metasilicate and also below the transition point between the said compatible crystalline metaborate and the crystalline metaborate of next 40 higher melting temperature.

CHESTER L. BAKER.